

Jan. 11, 1949.

F. A. LOWENHEIM

2,458,912

ELECTROPLATING OF TIN

Filed April 27, 1944

*Fig. 1.*



*Fig. 2.*



INVENTOR

Frederick A. Lowenheim

BY

Gifford, Deull, and Burgess  
ATTORNEY

## UNITED STATES PATENT OFFICE

2,458,912

## ELECTROPLATING OF TIN

Frederick A. Lowenheim, Plainfield, N. J., assignor  
to Metal & Thermit Corporation, New York,  
N. Y., a corporation of New Jersey

Application April 27, 1944, Serial No. 532,932

8 Claims. (Cl. 204—54)

**1**  
This invention relates to the improvement of aqueous alkaline stannate electroplating processes. It also relates to improving the anode efficiency of alkaline stannate tinplating cells. It also relates to anodes of greater efficiency in aqueous alkaline stannate electroplating baths.

In electroplating tin from alkaline stannate baths, those who practice the art have employed soluble anodes of pure tin and have regulated the variables such as the composition of the bath, the cathode current density, the anode current density and the caustic concentration so that the solution of tin from the anodes replenishes the tin content of the bath as the tin is deposited at the cathode. Those attempts are successful only within limits and can be used to produce only limited flexibility in control of the process.

Attempts have been made to improve the efficiency of such baths by increasing the free alkali content of the solution, but this has been accompanied by a lowering of the cathode efficiency. To counteract this lowered cathode efficiency the tin content of the bath has been raised. This series of measures does in fact permit the use of higher current densities, but they are accompanied by the disadvantage that they lead to the use of unduly high concentrations and to dragout losses which are uneconomical.

While the foregoing measures are effective to the extent indicated in connection with potassium stannate baths they are not useful for sodium stannate baths because of their limited cathode efficiency, the limited solubility of sodium stannate, and the much greater tendency of sodium stannate baths to precipitate insoluble tin compounds by hydrolysis.

High rates of cathode deposition have also been secured by increasing the ratio of anode area to cathode area, so that the cathode current densities remain high and the anode current densities remain relatively low, each of which is in the interests of efficiency. This modification has a limitation imposed upon it by geometrical configuration and mechanical design, for example in the continuous electrotinning of strip steel where in the mechanical features of the apparatus limit the area of anode.

It is an object of my invention to provide an anode for the electrolytic deposition of tin which will exhibit higher current efficiency than an anode of pure tin in any alkaline stannate plating bath without introducing harmful ingredients in the bath.

A second object of my invention is to increase

**2**  
the anode efficiency in alkaline stannate electroplating baths.

A third object of my invention is to improve the overall efficiency of potassium stannate electroplating cells and of sodium stannate electroplating cells.

A fourth object of my invention is to form tin anodes that will be of increased efficiency in electroplating cells.

**10** The objects of the invention are accomplished generally speaking by making an anode composed of tin alloyed with a small amount of aluminum and using it in alkaline stannate electroplating cells, particularly in potassium stannate electroplating cells.

The objects and nature of the invention will be more fully understood from a consideration of the specification and claims which follow:

The invention has particular application to the **20** tinplating of strip steel, which is carried out by passing a steel strip through a plating cell as a moving cathode. In that application of the invention the speed of electrodeposition is of the essence. In one important aspect of that process, **25** a large tank is provided with a series of anodes having faces relatively close together, and an aqueous alkaline stannate bath. Between the faces of the anodes the moving steel strip, connected in the cell as a cathode, is passed at a rate such that when it emerges from the cell it is perfectly plated. In order that this plating **30** shall not vary in quality it is necessary that the bath operate with uniformity. For most economical results it is also desirable that the steel **35** shall travel with the high speed offered by the cathode efficiency of a potassium stannate bath, but in some cases this cannot be continuously maintained economically because of the relative inefficiency of the anodes. It is economically **40** impractical to alter the design of the cells to accommodate anodes of sufficient oversize to achieve any satisfactory improvement in operating conditions. When it is realized that each of the anodes used in such cells weighs in the **45** thousands of pounds, this will be readily understood. By the practice of my invention the foregoing difficulties are overcome.

According to my invention as applied to strip plating with an electrolytic bath containing **50** alkali stannate and alkali hydroxide in selected and efficient concentration, the anodes are placed in the bath and connected to a source of current, the steel strip which is to be plated is passed between the anodes, with its surfaces a short distance from the faces

of the anodes, and is connected to the negative pole of the source of current. The current is then turned on and the current density increased until that critical point is reached at which a great increase in voltage is employed in order to film the anodes. After the anodes have been filmed the voltage and current density are reduced to proper operating conditions. The speed of the cathode through the bath is then adjusted to the highest speed which can be efficiently employed, considering the weight of tin it is desired to deposit on the surface of the cathode. The temperature of the bath, the current density on the anode, the current density on the cathode, and the concentration of alkali hydroxide and tin in the bath are maintained at the most favorable figures.

If such a cell be operated with pure tin anodes, and an identical cell be operated under identical conditions but using my improved anodes, it will be found that practicable working anode current densities in the case of the improved anodes are almost doubled in many instances and in all cases are substantially increased. Speeds at which satisfactory plating can be carried out are increased in proportion.

The tin-aluminum alloys may be prepared by making a master alloy according to a selected formula, containing, for instance, 90% tin and 10% aluminum. When tin and aluminum are melted and uniformly mixed so that the aluminum is evenly distributed in the mass a substantially perfect alloy is produced which may be subdivided to make the anodes. In making the anodes, calculated amounts of this master alloy are introduced into a melt of pure tin and cast into the desired form of the anode. As little as one-tenth of one per cent of aluminum when added to the pure tin of the anode has a markedly beneficial effect on the anode efficiency. The anode efficiency is further increased by increasing its aluminum content toward 1%. Anodes containing more than about 1% of aluminum also show beneficial effects but the increase of aluminum content beyond about 1% produces little increase in efficiency.

The forgoing technique of alloy manufacture is satisfactory but not essential, since the anode can be prepared by melting pure tin and mixing with it the percentage of aluminum desired in the anode.

In order to demonstrate the improvement which is attained by this invention the reports of certain experiments are set forth hereinafter, and the results are plotted on the graphs in the accompanying drawings. In the drawings the graphs show anode efficiency in per cent as the vertical axis and anode current density in amperes per square foot as the horizontal axis. Electrode efficiency is the ratio of actual metal dissolved or deposited compared with the metal theoretically dissolved or deposited according to Faraday's law.

Fig. 1 shows in the upper line the efficiency of a tin anode containing 0.72% aluminum, and in the lower line the relative efficiency of a pure tin anode.

Fig. 2 is a similar graph showing in the top line the efficiency of several anodes containing from 0.75% to 2% aluminum, in the intermediate lines the efficiency of anodes of 0.5%, 0.25% and 0.1% aluminum respectively, and in the lower line the relative efficiency of a pure tin anode.

The relation of the figures to the following examples is explained in the examples.

### Example 1

Figure 1 shows the results of tests on pure tin and on 0.72% aluminum anodes respectively in a potassium stannate bath of the following composition maintained at 90° C.:

Sn ----- 40.5 g./l. (.34 M./l.)  
Free KOH ----- 11.0 g./l. (0.2 M./l.)

The improvement made possible by the use of the aluminum alloy is brought out by the following comparative table showing the anode current densities obtainable for a given anode efficiency as read off the curves:

| Efficiency      | A<br>Anode Cur-<br>rent Pure Sn | B<br>Density<br>0.72% Al | Ratio: $\frac{B}{A}$ |
|-----------------|---------------------------------|--------------------------|----------------------|
| <i>Per cent</i> |                                 |                          |                      |
| 100             | 19                              | 44                       | 2.3                  |
| 95              | 25                              | 52                       | 2.1                  |
| 90              | 29                              | 60                       | 2.1                  |
| 85              | 33                              | 68                       | 2.1                  |
| 80              | 38                              | 76                       | 2.1                  |
| 75              | 40                              | 84                       | 2.1                  |
| 70              | 43                              | 92                       | 2.1                  |

On the average, the table shows that the anode current density may be more than doubled by the use of 0.72% aluminum alloyed with the tin.

Figure 2 shows the effect that changing the aluminum content of the anode has on the anode efficiency in a potassium stannate bath of the same composition as used above.

Similar improvement has been observed in baths of other concentrations and temperatures.

### Example 2

Tests of the new anodes were also run in sodium stannate baths, which were also improved thereby. The results shown in the following table were obtained with anodes containing 0.5% aluminum in a sodium stannate bath of the following composition at 90° C.:

Sn ----- 40 g./l. (.34 M./l.)  
Free NaOH ----- 7.5 g./l. (.19 M./l.)

50

| Efficiency      | A<br>Anode Cur-<br>rent Pure Sn | B<br>Density<br>0.56% Al | Ratio: $\frac{B}{A}$ |
|-----------------|---------------------------------|--------------------------|----------------------|
| <i>Per cent</i> |                                 |                          |                      |
| 100             | 27                              | 29                       | 1.07                 |
| 95              | 32                              | 40                       | 1.25                 |
| 90              | 37                              | 51                       | 1.38                 |
| 85              | 42                              | 57                       | 1.35                 |
| 80              | 45                              | 62                       | 1.38                 |
| 75              | 48                              | 66                       | 1.37                 |
| 70              | 50                              | 70                       | 1.40                 |

The improvement in the sodium stannate bath is shown to be approximately 35-40% omitting the first line of the table.

### Example 3

The following four tests show that the addition of aluminum increases the anode efficiency regardless of the solution compositions. All tests were run at 90° C.:

(a) Solution:

Sn ----- 31 g./l. (.26 M./l.)  
Free KOH ----- 8.5 g./l. (.15 M./l.)

75

## Tank 2—0.6% Al anodes:

Average amperes, 95

Total ampere hrs. 1680

Average anode current density, 110 A/SF

5 Average anode area, 0.85 sq. ft.  
Overall anode efficiency, 89%

| Efficiency      | A<br>Anode Cur-<br>rent Pure Sn | B<br>Density<br>.92% Al | Ratio: B<br>A |
|-----------------|---------------------------------|-------------------------|---------------|
| <i>Per cent</i> |                                 |                         |               |
| 100             | 16                              | 27                      | 1.69          |
| 95              | 20                              | 32                      | 1.60          |
| 90              | 23                              | 35                      | 1.52          |
| 85              | 29                              | 39                      | 1.35          |
| 80              | 32                              | 42                      | 1.32          |
| 75              | 35                              | 46                      | 1.32          |
| 70              | 38                              | 50                      | 1.32          |

## (b) Solution:

Sn ----- 41 g./l. (.35 M./l.)  
Free KOH ----- 20 g./l. (.36 M./l.)

15

| Efficiency      | A<br>Anode Cur-<br>rent Pure Sn | B<br>Density<br>.92% Al | Ratio: B<br>A |
|-----------------|---------------------------------|-------------------------|---------------|
| <i>Per cent</i> |                                 |                         |               |
| 100             | 24                              | 40                      | 1.67          |
| 95              | 31                              | 50                      | 1.62          |
| 90              | 36                              | 67                      | 1.36          |
| 85              | 40                              | 75                      | 1.38          |
| 80              | 44                              | 85                      | 1.33          |
| 75              | 48                              | 91                      | 1.39          |
| 70              | 53                              | 97                      | 1.33          |

## (c) Solution:

Sn ----- 41 g./l. (.35 M./l.)  
Free KOH ----- 29 g./l. (.52 M./l.)

15

20

| Efficiency      | A<br>Anode Cur-<br>rent Pure Sn | B<br>Density<br>1.28% Al | Ratio: B<br>A |
|-----------------|---------------------------------|--------------------------|---------------|
| <i>Per cent</i> |                                 |                          |               |
| 100             | 33                              | 60                       | 1.82          |
| 95              | 41                              | 84                       | 2.05          |
| 90              | 46                              | 97                       | 2.10          |
| 85              | 53                              | 110                      | 2.07          |
| 80              | 59                              | 120                      | 2.03          |
| 75              | 64                              | 131                      | 2.04          |
| 70              | 69                              | 137                      | 1.98          |

## (d) Solution:

Sn ----- 81 g./l. (.68 M./l.)  
Free KOH ----- 46 g./l. (.87 M./l.)

30

35

40

| Efficiency      | A<br>Anode Cur-<br>rent Pure Sn | B<br>Density<br>.56% Al | Ratio: B<br>A |
|-----------------|---------------------------------|-------------------------|---------------|
| <i>Per cent</i> |                                 |                         |               |
| 100             | 39                              | 75                      | 1.92          |
| 95              | 50                              | 108                     | 2.16          |
| 90              | 59                              | 117                     | 1.98          |
| 85              | 68                              | 127                     | 1.87          |
| 80              | 76                              | 134                     | 1.76          |
| 75              | 86                              | 142                     | 1.65          |
| 70              | 92                              | 152                     | 1.65          |

## Example 4

Tests were run on a solution having the following composition:

Sn ----- 61 g./l. (.52 M./l.)  
Free KOH ----- 36 g./l. (.64 M./l.)

Temperature 90° C.

In one tank, tin anodes in the shape of rods were hung and in the other, tin-aluminum (0.6% aluminum) alloy anodes of the same shape.

## Tank 1—Sn anodes:

Average amperes, 85

Total ampere hrs. 1450

Average anode current density, 68 A/SF

Average anode area, 1.25 sq. ft.

Overall anode efficiency, 90%

45

50

55

60

65

70

75

78

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

through an aqueous alkaline stannate bath the step of improving the anode efficiency of the bath which comprises employing an anode consisting essentially of tin alloyed with about 0.1 to 2% of a metal of the class consisting of aluminum, gallium and manganese.

2. Process according to claim 1 in which the bath is an aqueous potassium stannate bath.

3. Process according to claim 1 in which the bath is an aqueous sodium stannate bath.

4. Process according to claim 1 in which said metal is aluminum.

5. Process according to claim 1 in which said metal is gallium.

6. Process according to claim 1 in which said metal is manganese.

7. In the process of electroplating tin by passing an electric current from an anode to a cathode through an aqueous potassium stannate bath, the step of improving the anode efficiency of the bath which comprises employing an anode consisting essentially of tin alloyed with about 1% aluminum.

5 8. The process of electroplating tin which comprises passing an electric current from an anode consisting of tin alloyed with from 0.1 to 2% of a metal of the class consisting of aluminum, gallium and manganese through an aqueous alkaline stannate bath to a moving steel strip connected as a cathode in the bath.

FREDERICK A. LOWENHEIM.

10

#### REFERENCES CITED

The following references are of record in the file of this patent:

#### UNITED STATES PATENTS

| 15 | Number    | Name     | Date          |
|----|-----------|----------|---------------|
|    | 1,466,126 | Fink     | Aug. 28, 1923 |
|    | 2,078,868 | Oplinger | Apr. 27, 1937 |

#### OTHER REFERENCES

20 Aufbau der Zweistofflegierungen, by Hansen, pages 153-155, 1936.

Transactions American Electrochemical Society, vol. 45, pages 431-440, 1924.